

## UNITED STATES PATENT OFFICE

MEYRL M. FROST, OF CAPAC, MICHIGAN

## PRODUCTION OF FIBER ARTICLES

No Drawing. Application filed August 20, 1927, Serial No. 214,441. Renewed May 1, 1929.

The present invention relates to the production of articles of compressed fibrous materials and particularly to a process of producing such articles and the articles produced thereby.

5 Among the objects of the invention is an article of manufacture which is extremely compact, tough, waterproof and capable of taking an excellent finish.

10 Other objects will readily appear to those skilled in the art upon reference to the following description.

Heretofore, such articles of manufacture as chair or toilet seats, doors, boxes and the like have been usually made of wood pieces glued or otherwise secured together. Wood has been considered the only suitable material because of its plentifulness and also because of its low heat conductivity. However, due to its property of absorbing moisture, it is difficult if not impossible to build up an article, such as a toilet seat, from pieces of wood glued together and have the pieces adhere permanently.

25 The present process produces an article that is not built up of pieces but is of homogeneous composition, water proof and has all of the advantageous properties of wood.

The process is carried out by first forming 30 a fluent pulp of fibrous material, such as ground wood pulp or pulp of rag fiber, waste-paper, hemp, jute or even asbestos. The pulp is beat up to a liquid form by adding a solution of casein and borax thinned down 35 with water to the desired consistency. This pulp after heating is put into suitable dies and pressed under the desired pressure preferably 300 to 500 pounds per square inch depending on the article to be formed. This 40 article is then removed from the dies and allowed to dry. After drying the article is then dipped in a bath of formaldehyde which acts chemically upon the casein and makes the article practically water proof.

45 Now having described this invention and the preferred form of embodiment thereof, it is to be understood that the said invention is to be limited not to the specific details herein set forth but only by the scope of the 50 claims which follow.

I claim:

1. The process of producing homogeneous fiber articles which consist in forming a pulp of the fiber in finely divided conditions with water mixing with said pulp casein and borax 55 expressing said water therefrom, drying and subjecting the molded article to an impregnation treatment with formaldehyde.

2. The process of producing homogeneous fiber articles which consist in forming a pulp 60 of the fiber in finely divided conditions with water mixing with said pulp casein and borax expressing said water and molding the fiber under a pressure of up to 600 pounds per square inch drying and subjecting the molded 65 article to an impregnation bath with formaldehyde.

3. An article of manufacture comprising a hard tough body of finely divided organic fiber and casein and borax with at least a 70 superficial impregnation of formaldehyde.

MEYRL M. FROST.

75

80

85

90

95

100